

## UNITED STATES PATENT OFFICE

2,534,316

## TREATMENT OF WOOL TO INCREASE ITS HARSHNESS AND DECREASE ITS LUSTER

Stuart E. Swanson, Suffield, Conn., assignor to Bigelow-Sanford Carpet Co., Inc., Thompsonville, Conn., a corporation of Massachusetts

No Drawing. Application January 13, 1948,

Serial No. 2,138

3 Claims. (Cl. 8-95)

1

The present invention relates to the treatment of wool to improve its physical properties and more particularly to a treatment which will enhance the harshness of the wool while at the same time decreasing its lustre.

In the manufacture of pile fabric floor covering by the established operations peculiar to this field, including the carding, spinning, dyeing, etc. of the fiber, it is necessary that the wool have a certain harshness of texture. In addition, the wool in the pile tufts of the completed product, should in many cases have a low degree of lustre.

B. A.-type wool is so deficient in harshness that it has not been possible to process it into carpets or rugs by the established procedure and with the equipment presently installed in carpet manufacturing plants, which procedure and equipment operate successfully with the conventional, harsher, carpet wools. Because of the soft, slippery, silk-like nature of the B. A.-type wool fibers, great care and constant attention must be exercised throughout the processing of the wool and the yarn and the weaving thereof. The resulting product is in a sense a handmade article and commercial production by the established practice is not feasible.

It is an object of the present invention to provide a process for harshening and deflustering B. A.-type wools thereby to extend their use in the manufacture of pile fabric floor coverings.

By the present invention I provide a process for so modifying these B. A.-type wools that the harshness of the fiber is increased to such an extent that the modified wool may be manufactured into pile fabric floor covering on a commercial scale by the conventional procedure and apparatus with only normal attention during the processing. It is possible to manufacture on a commercial basis pile fabric floor coverings consisting entirely of B. A.-type wools modified by my process. The treatment of my invention also decreases the lustre of the wool.

I have discovered that by treating these soft, silk-like, lustrous, slippery B. A.-type wools with a solution of barium oxide or barium hydroxide, preferably in a bath containing the barium compound, and then treating the wool with sulfuric acid, the fibers of these wools are rendered harsher so that they may be handled by the methods conventional in the carpet manufacturing industry, in which methods the harsher wools from other parts of the world are used. Also, at the same time, the lustre of said fibers, which is undesirable in conventional domestic rugs and carpets, is decreased.

2

The following is given as an example of my process:

A batch of raw B. A. wool stock weighing about 900 pounds is immersed in about 4,000 gallons of a cold aqueous solution containing 45 pounds of barium oxide. The solution is brought to the boil and maintained at the boiling point for about 10 minutes, following which the solution is drained off. The treated wool is then thoroughly rinsed by circulating tap water in the kettle containing the wool and draining that water off. This rinse removes excess barium compound. The kettle, still containing the wool, is again filled with tap water and sulfuric acid is added in an amount sufficient only to make the bath slightly acid. This makes the barium compound in the wool insoluble and thus fixes it therein. Thereafter, the wool is removed from the kettle and dried. The resulting modified wool can be processed into pile fabric floor covering by the conventional procedures employed with the usual carpet wools with no more than normal care and attention.

The barium oxide of the foregoing example may be replaced partly or entirely by barium hydroxide.

The pH of the barium solution, I have found, should be in the range 7.0 to 12.0.

I prefer that the bath be kept at the boil during the treatment with the barium compound, as in the foregoing example, and that the wool be kept in the barium solution at or near the boil for a period of 10 to 20 minutes. However, satisfactory modification of the wool may be obtained at lower temperatures by allowing the wool to remain standing in the bath for correspondingly longer periods of time. In this case, the barium oxide or barium hydroxide may be incorporated in the bath in the same proportion used with the boiling bath.

If the wool is to be colored, it may be acid dyed after it has been modified by the treatment of this invention.

I have found that the proportion of barium compound present in the treating liquid may be varied over a substantial range depending upon the degree of modification to be imparted to the wool and upon the temperature and the duration of the treatment. Amounts of the barium compound or compounds ranging from about 2% to 10%, by weight of the wool, preferably about 5%, have been found advantageous.

Another mode of treatment is to treat the wool with a barium compound as a continuous operation in a moving stream of liquid. Thus the wool may be treated as it is subjected to the rinsing

operation which normally follows the scouring operation in the preparation of wool fibers for use in pile fabric floor coverings. This procedure is particularly useful with wools which are not to be dyed but are to be manufactured into yarn of their natural color. In many cases the rinsing following the scouring operation is carried out with water at a temperature at about 140°-160° F., although rinsing at any temperature between room temperature and the boiling point may be employed. The barium compound content of the rinse bath should approximate 1% to 8%, preferably about 1%, of the volume of the bath. The wool is passed through the rinsing tank in a continuous operation and the barium compound or compounds therefore must be continually supplied to the tank to maintain the desired concentration therein. For this purpose any appropriate, constant-rate feeding means may be employed. Following said rinse the wool is treated with a dilute bath of sulfuric acid approximating 0.1% to 1.0%, preferably 0.3%, based on the volume of the bath.

The treatment of the present invention is most useful when applied to the B. A.-type wools because, in this case, it serves to convert a wool which can be used only in minor proportions, if at all, for the manufacture of pile fabric floor coverings, into a wool which can be used substantially in the same way as the conventional carpet wools. However, my treatment is also useful with these conventional carpet wools to decrease their lustre and to enhance their harshness to render them amenable to processing into pile fabric floor coverings by the established procedures and equipment. The improvement in these properties, however, is not as great in the case of the conventional carpet wools as it is with the B. A.-type wools. The treatment is also useful with mixtures of wools of different types.

Wool modified by my process may be spun into yarn which may then be woven as the pile of pile fabric floor coverings, notwithstanding the fact that the original stock was largely or entirely a B. A.-type wool which inherently is incapable of being processed on the conventional carpet manufacturing apparatus. Such pile has a coarse harsh texture and a lack of lustre far different from the texture and lustre of untreated B. A.-type wools and comparable with the texture and lustre of the conventional carpet wools. Raw B. A.-type wool stock modified by my process may be mixed with conventional carpet wools in all proportions to give a wool mixture suitable for use in forming the pile of pile fabric floor coverings.

By the term "B. A.-type wool," as used herein, I mean wool having the characteristics of "B. A. wool" as regards its soft, slippery nature, its lustre and its lack of harshness and fullness as contrasted with the conventional carpet wools. I use the term "B. A. wool" in its ordinary meaning in the trade, i. e., wool from the Lincoln-

type sheep as grown in South America. The "B. A.-type" wools available today consist primarily of B. A. wool, and wool from the Lincoln-type sheep as grown in New Zealand.

Although the above specific examples of my process, given by way of illustration and not of limitation, relate to procedures in which the wool is immersed in a bath of the barium compound, it is not intended thereby to exclude other ways of applying the treating solution to the wool, such as by sprinkling, spraying, etc.

I claim:

1. The process for imparting to B. A.-type wool the property of harshness requisite for conversion of the wool by standard procedures into pile fabric floor covering, and for decreasing its lustre, which consists essentially in wetting the wool with a solution having a pH between 7.0 and 12.0 and containing a barium compound selected from the class consisting of barium oxide and barium hydroxide, and thereafter treating the wool with sulfuric acid.

2. The process for imparting to B. A.-type wool the property of harshness, requisite for conversion of the wool by standard procedures into pile fabric floor covering, and for decreasing its lustre, which consists essentially in immersing the wool for 10 to 20 minutes in a boiling aqueous solution having a pH between 7.0 and 12.0 and containing 2% to 10% by weight of the wool of barium oxide, and thereafter treating the wool with sulfuric acid.

3. The process for imparting to B. A.-type wool the property of harshness requisite for conversion of the wool by standard procedures into pile fabric floor covering, and for decreasing its lustre, which consists essentially in immersing the wool for 10 to 20 minutes in a boiling aqueous solution having a pH between 7.0 and 12.0 and containing 2% to 10% by weight of the wool of barium hydroxide, and thereafter treating the wool with sulfuric acid.

STUART E. SWANSON.

#### REFERENCES CITED

The following references are of record in the file of this patent:

#### UNITED STATES PATENTS

| Number    | Name    | Date          |
|-----------|---------|---------------|
| 1,839,979 | Lorimer | Jan. 5, 1932  |
| 1,947,024 | Slagle  | Feb. 13, 1934 |
| 2,152,182 | Ellis   | Mar. 28, 1939 |

#### FOREIGN PATENTS

| Number  | Country       | Date          |
|---------|---------------|---------------|
| 383,149 | Great Britain | Nov. 10, 1932 |

#### OTHER REFERENCES

60 Gooch et al., "Outlines of Inorganic Chemistry," Macmillan Co., New York, 1905, page 252. (Copy in Patent Office Scientific Library.)